

## UNITED STATES PATENT OFFICE

2,375,626

## SOAP ANTOXIDANT

Elmer W. Cook, New York, N. Y., assignor to  
 American Cyanamid Company, New York,  
 N. Y., a corporation of Maine

No Drawing. Application March 2, 1944,  
 Serial No. 524,780

2 Claims. (Cl. 260—398.5)

This invention relates to an improvement in soap and soap products, and more particularly to the stabilization of soap against discoloration and rancidity upon storage. By "soap" I mean ordinary commercial soap, which is an alkali metal salt of a fat acid such as is obtained by the saponification of vegetable or animal fats of the type of tallow, coconut oil and the like.

I have found that the biguanide and hydrocarbon-substituted biguanide salts of p-tertiary amylophenyl phosphoric acids are improved soap stabilizers and will prevent discoloration and rancidity in soap to a marked degree. Accordingly, my invention consists in the stabilization of soap against discoloration and rancidity by incorporating therein small but effective amounts of a biguanide p-tertiary amylophenyl phosphate. I have found that a high degree of stabilization is obtained when amounts on the order of 0.01-0.5% of my new stabilizer are used, based on the weight of the soap.

Biguanide itself and such substituted biguanides as mono-orthotolyl biguanide, mono-phenyl biguanide, mono-xylyl biguanide and bi-phenyl biguanide have hitherto been used as soap stabilizers, either as such or in the form of salts with hydrochloric acid. However, the hydrochlorides and other simple salts of these biguanide compounds are no better stabilizers than are the biguanides themselves. It is therefore quite surprising to find that the p-tertiary amylophenyl phosphate salts of these biguanides possess improved soap stabilizing properties, for the alkali metal and other simple salts of p-tertiary amylophenyl phosphate possess little or no soap stabilizing properties.

The p-tertiary amylophenyl phosphoric acids are prepared by reacting p-tertiary amylophenol with P<sub>2</sub>O<sub>5</sub>. Either the mono- or the diester may be prepared in this manner and used to form a biguanide or hydrocarbon-substituted biguanide salt. Preferably I prepare a mixture of mono- and diesters by heating 1 mole of phosphorous pentoxide with 3 moles of p-tertiary amylophenol with stirring for 1 hour. The reaction product may then be added to a biguanide such as biguanide itself, mono-phenylbiguanide or mono-biphenylbiguanide in alcohol solution, preferably with the application of heat to complete the salt formation.

In practicing my invention any biguanide which in itself possesses soap stabilizing properties may be combined with p-tertiary amylophenyl phosphoric acid to form a salt, and in all cases it will be found that the stabilizing properties of the biguanide are improved. I prefer, however, to use the p-tertiary amylophenyl phosphate salts of the mono-aryl biguanides, and particularly the monophenyl and substituted monophenyl biguanides such as those enumerated above. These

preferred compounds are preferably incorporated into the soap in amounts of about 0.01-0.2%, based on the weight of the soap, 0.1% being a suitable quantity. My invention will be described in greater detail by reference to the following specific example.

## Example

Fine white milled soap, having a neutralization number of 0.29, was ground and 0.1% of stabilizer was incorporated by adding 0.015 gram of the stabilizer to 15 grams of the soap. 150 cc. of hot, oxygen-free distilled water was then added and the mixture stirred with heating until the entire mass was dissolved. The solution was poured into a flat dish and cooled to a gel, which was dried to 10% moisture content. Three of the dried films were then united by pressure into a cylindrical cake about  $\frac{3}{8}$  inches in thickness, using a hydraulic press and a pressure of 2160 pounds per square inch for 15 minutes. The resulting soap bar was placed in a jar fitted with a screw cap. A number of samples containing various soap antioxidants were prepared in this manner, as well as a blank sample containing no stabilizer.

The jars were closed and placed in a constant temperature oven maintained at 80° C. for accelerated aging, and the samples were removed each day and inspected for discoloration and rancidity. Discoloration of the aged soap bars was determined by measuring absorption in the yellow end of the spectrum at 4200 Å, using a recording spectrophotometer for this purpose. In the following table T<sub>0</sub> equals percent reflection before aging and T<sub>1</sub> equals percent reflection after aging. In all cases the results given were obtained after an aging time of seven days.

| 40 | Compound                                       | $\frac{T_0}{T_1}$ |
|----|------------------------------------------------|-------------------|
|    | None.                                          | 0.341             |
|    | Na p-tert. amylophenyl phosphate.              | 0.306             |
|    | Phenylbiguanide hydrochloride.                 | 0.207             |
|    | Phenylbiguanide.                               | 0.140             |
| 45 | Phenylbiguanide p-tert. amylophenyl phosphate. | 0.108             |

## What I claim is:

1. Soap stabilized against discoloration and rancidity by the presence therein of stabilizing amounts of a biguanide salt of a p-tertiary amylophenyl phosphoric acid, said soap being an alkali metal salt of a fat acid.
2. Soap stabilized against discoloration and rancidity by the presence therein of stabilizing amounts of a mono-phenyl biguanide salt of a p-tertiary amylophenyl phosphoric acid, said soap being an alkali metal salt of a fat acid.

ELMER W. COOK.